

## 1

3,026,171

## MANUFACTURE OF RAYON

Nikolaus Augustin Schonfeldt, Molndal, and Kurt Helmut Grunewald, Goteborg, Sweden, assignors, by mesne assignments, to American Enka Corporation, Enka, N.C., a corporation of Delaware

No Drawing. Original application Mar. 23, 1953, Ser. No. 344,182. Divided and this application Sept. 28, 1959, Ser. No. 842,575

5 Claims. (Cl. 18—54)

This application is a division of our copending application Serial No. 344,182, filed March 23, 1953, and now abandoned.

The present invention relates to the manufacture of viscose rayon yarns, films and the like, and more particularly to the production of rayon in the presence of a quaternary ammonium compound.

In recent years, it has been determined that improved rayon yarns, films and the like could be manufactured by the use of modifiers that retard the regeneration processes in the viscose and thereby permit higher stretches which improved both the strength and fatigue. Some of these modifiers have been described in U.S. Patent Nos. 2,535,044, 2,535,045, and 2,536,014.

It is therefore an object of the present invention to provide a process for the manufacture of rayon yarns, films, and the like of improved strength and fatigue.

Another object of this invention is to provide a process for the manufacture of rayon in which the filaments have improved stretchability.

An additional object of this invention is to provide a process for the manufacture of rayon wherein spinneret incrustation is inhibited.

A further object of this invention is to provide a process for the manufacture of rayon wherein the filterability of the viscose is improved.

A still further object of this invention is to provide a process for the production of viscose of improved clarity.

It is an additional object of this invention to provide an improved viscose spinning solution.

These and other objects are accomplished by incorporating into the viscose at some stage in the processing a surface active, quaternary ammonium compound of the general formula:



wherein R is an aliphatic radical containing at least 8 carbon atoms, R' is a radical selected from the group consisting of oxyalkylene or polyoxyalkylene radicals, R'' is an alkyl radical having not more than 2 carbon atoms, and X is an innocuous anion consisting of or containing, e.g., a halogen, a  $\text{SO}_4\text{H}$  group and a  $\text{SO}_4\text{CH}_3$  group.

These compounds may be prepared by quaternizing a compound of the following formula:



wherein R is an aliphatic radical containing at least 8 carbon atoms and R' is a radical selected from the group consisting of oxyalkylene and polyoxyalkylene radicals. In the preferred compounds, R should be an aliphatic radical having 8 to 20 carbon atoms such as octyl, dodecyl, hexadecyl, and octadecyl.

The compound preferably contains 3 to 30 oxyalkylene radicals, but it may contain more or less. The oxyalkylene radical normally will be ethylene oxide, but it

## 2

may also be propylene oxide or substituted ethylene oxides.

The quaternization of these compounds may be, as for example, by condensation with alkyl halides such as ethyl chloride, or by reaction with an alkyl sulfate such as dimethyl sulfate or diethyl sulfate.

These quaternary ammonium compounds may be added at any stage of the process of manufacturing regenerated cellulose yarns. Thus it is possible to obtain improvements in this process by adding these compounds to the dissolving liquor, to the viscose solution, to the carbon disulfide during xanthation, to the steeping liquor, to the alkali cellulose spinning solution, or to the coagulating spinbath.

10 It is possible by the use of these compounds to improve the filterability and clarity of the viscose. It is also possible to increase the amount of stretch to which the filaments may be subjected during coagulation. In addition, they permit the production of a more uniform fiber.

20 Such quaternary ammonium compounds also inhibit the formation of spinneret incrustations as well as the inhibition of the formation of craters on the spinneret. In addition, it has been found that these compounds do not foam, thereby making them particularly adaptable in the process.

25 These results are obtained by choosing the proper compound for the desired improvements. Thus the selection of the various radicals mentioned above, as well as the point in the processing at which the material is used, depends upon the desired improvements. Each compound is not necessarily limited to improving one characteristic of the process but may improve several. For example, one that improves viscose filterability may also inhibit spinneret incrustations.

30 35 Such compounds, depending upon their composition, may be soluble or dispersible in 18-20% sodium hydroxide and others may be soluble or dispersible in the spinning bath. These properties depend upon the compounds used in their manufacture as well as the method of production. These compounds may be liquids or solids, which also depends upon their composition.

40 45 In some cases, it may be desirable to use these compounds in conjunction with other agents. Thus if they are used for emulsification, it may be desirable to use an emulsifying agent in combination with the quaternary ammonium compound.

These compounds may be added to the process in varying amounts, depending upon the desired result. Thus, it is possible to use an amount varying from 0.045% to 0.09%, based on the weight of the viscose. Other amounts may also be used.

50 55 The following examples will illustrate the various improvements obtained by the use of these quaternary ammonium compounds. These examples are included merely for the purpose of illustration and are not intended as limiting the scope of this invention.

## Example I

60 Lauryl amine was condensed with 4 moles of ethylene oxide and the condensation product was reacted with dimethyl sulfate to obtain a quaternary ammonium compound of the formula:



65 70 A dispersion of this product was prepared in 20% sodium hydroxide so that the dispersion contained 0.2 g. of this product. This compound increased the reactivity of the alkali cellulose.

## Example II

Stearyl amine was condensed with 20 moles of ethylene oxide and the condensation product was reacted with dimethyl sulfate to obtain a compound of the formula:



wherein  $y+z$  equals 20. This product in an amount of 0.5 g. per liter of viscose (about 0.045% based on the weight of the viscose) improves the clarity of the viscose and at the same time inhibits clogging of the spinnerets in the spinbath.

## Example III

Hexadecyl amine was condensed with 10 moles of propylene oxide and the resulting condensation product was reacted with dimethyl sulfate to obtain the quaternary ammonium compound of the formula:



wherein  $y+z$  equals 10. One part of this compound per 1000 parts of  $\text{CS}_2$  was added to the  $\text{CS}_2$  with a resulting improvement in emulsion xanthation.

## Example IV

Lauryl amine was condensed with 5 moles of ethylene oxide and the condensation product was reacted with dimethyl sulfate to obtain a compound of the formula:



wherein  $y+z$  equals 5. One gram of this compound per liter of the coagulating spinbath inhibited the formation of spinneret craters.

The foregoing examples illustrate that the quaternary ammonium compounds of this invention may be used in various ways to improve the processing of viscose yarn as well as improving the yarn itself.

The foregoing description is intended for the purpose of illustration, it being understood that departures from and modifications of this description may be made without departing from the spirit and scope of this invention which is to be limited only by the following claims.

The foregoing examples illustrate that the quaternary ammonium compounds of this invention may be used in various ways to improve the processing of viscose yarn as well as improving the yarn itself.

The foregoing description is intended for the purpose of illustration, it being understood that departures from

and modifications of this description may be made without departing from the spirit and scope of this invention which is to be limited only by the following claims.

What is claimed is:

5. In the manufacture of viscose yarn wherein a viscose solution is extruded through minute orifices into a coagulating spinbath to form filaments therefrom, the step which comprises spinning the viscose filaments in the presence of at least 0.045%, based on the weight of the viscose, of a quaternary ammonium compound represented by the following formula:



wherein R is an aliphatic hydrocarbon radical containing at least 8 carbon atoms,  $\text{R}'$  is an alkylene radical having from 2 to 3 carbon atoms,  $\text{R}''$  is an alkyl radical having from one to two carbon atoms, X is a halogen, and 10 x and y are integers having a sum total varying between 3 and 30.

20 2. In the manufacture of viscose yarn according to claim 1, wherein R is an aliphatic radical containing 12-20 carbon atoms.

25 3. In the manufacture of viscose yarn according to claim 1, wherein  $\text{R}''$  is a methyl group.

4. In the manufacture of viscose yarn according to claim 1, wherein  $\text{R}'$  is an alkylene radical having 2 carbon atoms.

30 5. In the manufacture of viscose yarn wherein a viscose solution is extruded through minute orifices into a coagulating spinbath to form filaments therefrom, the step which comprises spinning the viscose filaments in the presence of a sufficient amount of a quaternary ammonium compound to modify the properties of the yarn, said compound being represented by the following formula:



40 wherein R is an aliphatic hydrocarbon radical containing at least 8 carbon atoms,  $\text{R}'$  is an alkylene radical having from 2 to 3 carbon atoms,  $\text{R}''$  is an alkyl radical having from one to two carbon atoms, X is an anion selected from the group consisting of a halogen, an  $\text{SO}_4\text{H}$  group, and an  $\text{SO}_4\text{CH}_3$  group, and x and y are integers having a sum total varying between 3 and 30.

## References Cited in the file of this patent

## UNITED STATES PATENTS

2,759,975 Chiddix et al. ----- Aug. 21, 1956

### **Disclaimer**

3,026,171.—*Nikolaus Augustin Schonfeldt, Molndal, and Kurt Helmut Grunewald, Goteborg, Sweden. MANUFACTURE OF RAYON.* Patent dated Mar. 20, 1962. Disclaimer filed Apr. 9, 1962, by the assignee, *American Enka Corporation.*

Hereby disclaims the residual term of said Letters Patent from Mar. 7, 1978 until Mar. 20, 1979.

[*Official Gazette May 22, 1962.*]